

# UNITED STATES PATENT OFFICE.

FRITZ ARLEDTER, OF PERLEN, SWITZERLAND.

## MANUFACTURE OF RESINOUS SOAP.

SPECIFICATION forming part of Letters Patent No. 627,287, dated June 20, 1899.

Application filed December 21, 1897. Serial No. 662,889. (No specimens.)

*To all whom it may concern:*

Be it known that I, FRITZ ARLEDTER, engineer, a citizen of Switzerland, and a resident of Perlen, near Lucerne, Switzerland, have invented certain new and useful Improvements in Manufacture of Resinous Soap, of which the following is a specification.

This invention has been patented to me in Norway under date of November 22, 1897, 10 and in Germany under date of November 18, 1897, No. 95,416.

My invention relates to the manufacture of resinous soap containing unsaponaceous resin and which is particularly adapted for use as 15 paper-size in the manufacture of paper.

According to my invention I boil the mass under pressure while continually stirring the same, the contents being thereby substantially converted into liberated resin—that is 20 to say, for the boiling of the soap according to my invention only seven to ten per cent. of alkali is necessary as against ten to fifteen per cent. by the methods hitherto known. The chemically-free or so-called “liberated” 25 resin may amount to forty-five per cent. of the resinous soap as against twenty-five per cent., which has hitherto been the maximum. Acting on the theory of Dr. Würster—viz., that only liberated resin sizes paper—I have 30 succeeded in sizing paper with one and a half to two per cent. of resin—that is to say, one and a half to two kilograms of resin to one hundred kilograms of paper. The main feature of my invention consists, therefore, in 35 the large proportion of liberated resin and in

the microscopically-fine distribution of this resin, whereby a considerable saving over the sizing methods hitherto known is effected.

Among the advantages of my method of manufacture may be specially mentioned: 40 Considerably shorter duration of the boiling. The quantity of liberated resin may be raised to fifty per cent. without causing inconvenience by the dissolution of such resinous soap, such as deposit of undissolved resin, 45 obstruction of the piping, and of the paper-machine. By steady boiling uniform sizing is obtained, and I am enabled to size paper with one and a half to two per cent. of resin. A considerable saving is therefore obtained 50 over the hitherto-known methods.

Having now described my invention, what I claim as new, and desire to secure by Letters Patent, is—

The herein-described method of producing 55 a resinous soap containing unsaponaceous resin serviceable in the manufacture of paper as paper-size consisting in boiling under great pressure resin and a quantity of alkali not sufficient for the complete saponification of 60 the resin, substantially as described.

In testimony that I claim the foregoing as my invention I have signed my name, in presence of two witnesses, this 23d day of November, 1897.

FRITZ ARLEDTER.

Witnesses:

AXEL GOTTFRIED GRONN LAHN,  
JOSEFINE JOHNSEN.